

# UNITED STATES PATENT OFFICE.

BERTHOLD WUTH, OF BASEL, SWITZERLAND, ASSIGNOR TO SOCIETY OF CHEMICAL INDUSTRY IN BASEL, OF BASEL, SWITZERLAND.

## PROCESS OF PRODUCING DISCHARGE EFFECTS ON COLORED GROUNDS.

1,000,313.

Specification of Letters Patent.

Patented Aug. 8, 1911.

No Drawing.

Application filed April 13, 1910. Serial No. 555,188.

To all whom it may concern:

Be it known that I, BERTHOLD WUTH, doctor of philosophy, chemist, a subject of the King of Great Britain, and resident of 5 Basel, Switzerland, have invented a new Process of Producing Discharge Effects on Colored Grounds, of which the following is a full, clear, and exact specification.

This invention makes use of the fact that 10 organic ammonium compounds in presence of alkali have a decomposing action on the majority of organic dyestuffs. This is especially the case at higher temperatures and this behavior of the organic ammonium compounds can be applied in a suitable manner 15 for white or variegated discharge effects on colored grounds. If dyed cotton be printed with a mixture of alkali and an organic ammonium compound, such as dimethyl- 20 phenylbenzylammonium chlorid and afterward steamed, a white discharge effect is produced on the dyed goods. If the alkaline discharge be mixed with a dyestuff adapted to withstand the decomposing effect 25 of the organic ammonium compound, variegated discharge effects can be obtained. By application of the invention pure white discharges can be produced on light and medium dyeings without any other addition and 30 without subsequent treatment. For discharge effects on dark dyed grounds an addition of glucose is to be recommended.

The application of organic ammonium compounds in connection with discharges 35 for colored grounds has been already proposed, but not their application alone; it has merely been suggested that they should be added to printing colors which contain formaldehyde sulfoxylate in order to increase 40 the discharging action of the latter. (See Austrian patent specification No. 28437, dated March 15, 1906.) From this known method of discharging the invention differs in that the discharging effect is due solely 45 to the ammonium compound in complete absence of other discharging substances (such as hydrosulfite preparations). Particularly good results are obtained by using dimethyl-phenylbenzylammonium chlorid, although 50 other organic ammonium compounds may be used, such as trimethylphenylammonium chlorid, a tetra-alkylammonium chlorid or trimethylbenzylammonium chlorid, also such

ammonium compounds as are themselves dyestuffs, such as brilliant phosphin 5 G, 55 methyl green and the like.

The method may be applied to very different colored ground, but it is especially applicable to white and variegated discharge effects on dyeings obtained with vat dye- 60 stuffs.

The following examples illustrate the invention.

Example 1: For a white discharge, the fabric dyed with indigo, ciba violet, ciba 65 gray, helindon, orange or thio-indigo red, is printed with the following mixture:

|     |                                                   |
|-----|---------------------------------------------------|
| 300 | grams of gum solution (1:1).                      |
| 100 | " " dimethylphenylbenzylammonium chlorid. 70      |
| 100 | " " caustic soda lye of 40° Bé. specific gravity. |

After printing and drying, the goods are 75 steamed for 5 minutes in the Mather-Platt apparatus and then washed.

Example 2: For a red discharge, the fabric dyed with ciba blue 2 B or indigo M L B/6 B, is printed with the following 80 discharge mixture:

|     |                                                   |
|-----|---------------------------------------------------|
| 650 | grams of gum solution (1:1).                      |
| 150 | " " printing chrome red.                          |
| 100 | " " dimethylphenylbenzylammonium chlorid. 85      |
| 100 | " " caustic soda lye of 40° Bé. specific gravity. |

After printing and drying the treatment 90 is the same as described in Example 1.

Example 3: For a yellow discharge either of the following mixtures may be used:

(a)

|     |                                                                                                                                      |
|-----|--------------------------------------------------------------------------------------------------------------------------------------|
| 25  | grams of alizarin yellow 5 G. 95                                                                                                     |
| 165 | " " water.                                                                                                                           |
| 550 | " " gum solution (1:1).                                                                                                              |
| 100 | " " dimethylphenylbenzylammonium chlorid.                                                                                            |
| 100 | " " caustic soda lye of 40° Bé. 100 specific gravity.                                                                                |
| 60  | " " alkaline chrome mordant formed by a mixture of equal parts by weight of chrome acetate of 20° Bé. 105 and of soda lye of 40° Bé. |

(b)

600 grams of gum solution (1:1).  
100 " " dimethylphenylbenzylammonium chlorid.  
5 100 " " caustic soda lye of 40° Bé.  
specific gravity.  
200 " " cibanon yellow R of 10 per cent. strength.

10 What I claim is:

A process of producing white and variegated discharge effects on colored grounds, consisting in applying to the fabric an alka-

line printing mixture containing a discharging agent consisting solely of an organic ammonium compound, substantially as described.

In witness whereof I have hereunto signed my name this 14th day of March, 1910, in the presence of two subscribing witnesses.

BERTHOLD WUTH.

Witnesses:

GEORGE GIFFORD,  
AMAND RITTER.

Copies of this patent may be obtained for five cents each, by addressing the "Commissioner of Patents, Washington, D. C."